

# UNITED STATES PATENT OFFICE.

LEON McCULLOCH, OF WILKINSBURG, PENNSYLVANIA, ASSIGNOR TO WESTINGHOUSE ELECTRIC AND MANUFACTURING COMPANY, A CORPORATION OF PENNSYLVANIA.

## INSULATING MATERIAL.

1,386,008.

Specification of Letters Patent.

Patented Aug. 2, 1921.

No Drawing.

Application filed January 5, 1917. Serial No. 140,822.

*To all whom it may concern:*

Be it known that I, LEON McCULLOCH, a citizen of the United States, and a resident of Wilkinsburg, in the county of Allegheny and State of Pennsylvania, have invented a new and useful Improvement in Insulating Material, of which the following is a specification.

My invention relates to composite electrical insulating material consisting of a binder and flake material such as mica, and it has for its object to provide a composite material comprising a bond of a permanent nature, which shall be unaffected by heat within normal operating ranges and shall have no tendency to soften or shrink at such operating temperatures.

The bond which I prefer to employ for the purpose indicated consists of boron tri-  
20 oxid or some other oxygen compound of boron, with or without the addition of fillers or other ingredients. According to one method of applying my invention, mica flakes or mica splittings are built up into a plate of  
25 the required thickness, dry powdered boric acid or a boric acid compound, such as ammonium borate, being sprinkled between the successive layers of mica. The built-up plate is then baked under pressure at a tem-  
30 perature of 500° C. or less, thereby fusing and substantially dehydrating the boric acid and decomposing the ammonium borate, if the latter compound is employed, leaving fused boric oxid containing only small  
35 amounts of water and gases.

The foregoing process may be varied by applying boric acid or a boric acid compound, such as ammonium borate, in admixture with a liquid such as benzin or  
40 very thin varnish which does not dissolve the boric material, but only serves as a vehicle for spreading the boric material between the mica flakes; or the boric acid, ammonium borate or other boric acid compound may  
45 be applied in solution in water, alcohol or other solvent. The vehicle or the solvent will be driven off, either wholly or in part, by the subsequent heat treatment. Other ingredients may be added to the bonding  
50 material for increasing its adhesiveness or bulk, suitable materials for this purpose being shellac or other varnish gums and finely divided inorganic materials such as clays of the bentonite type, kaolin, metallic oxids  
55 and the like.

One bonding mixture which I have employed with good results is prepared by mixing dry boric acid or ammonium borate with a small amount of bentonite filler and working to a thin paste with a water solution of glycerin. The glycerin reacts with the boric acid present to form a sticky glyceryl borate which renders the entire mixture adhesive and effectually holds the mica flakes together during the building-up process. When heat  
60 is applied to the composite material, the glycerin is driven off, and the boric oxid which remains behind acts as the final bond.

Boric oxid imparts to composite materials containing it the property of softening at  
65 moderately elevated temperatures of the order of 500° C., but since the boric oxid does not become completely fluid except at temperatures several hundred degrees above this point, the composite material is entirely  
70 coherent at all temperatures ordinarily encountered in the operation of electrical apparatus. Boric oxid binders have the further advantage that they do not exert a de-  
75 structive fluxing action upon mica, as do many of the binding materials which have heretofore been employed for the purpose of making composite insulating materials.

It is to be understood that my invention is not restricted to the use of any particular  
80 proportions or materials except as indicated in the appended claims, and that the specific examples given herein are intended to be  
85 illustrative and may be widely modified without departing from the spirit and scope  
90 of my invention.

I claim as my invention:

1. A composite material comprising flake material and a lead free binder containing an oxygen compound of boron.
2. A composite material comprising flake material and a lead free binder containing boron trioxid.
3. A composite material comprising flake material and a lead free binder containing an oxygen compound of boron and a filler.
4. A composite material comprising flake material and a lead free binder comprising boron trioxid and a pulverulent filler.
5. A composite material comprising mica flakes or splittings held together by means of a lead free binder containing an oxygen compound of boron and a filler.
6. A composite material comprising mica flakes or splittings held together by means

- 2 of a lead free binder containing boron tri-  
oxid.
7. A composite material comprising mica  
flakes or splittings held together by means  
5 of a lead free binder containing boron tri-  
oxid and a pulverulent filler.
8. A process of making composite mate-  
rial that comprises associating flake material  
with an adhesive lead free binder containing  
10 an oxygen compound of boron, and applying  
heat and pressure to the said material.
9. A process of making composite mate-  
rial that comprises associating flake material  
with a binder formed by mixing boric acid,  
15 water and glycerin, and applying heat and  
pressure to the said material.
10. A process of making composite mate-  
rial that comprises superposing mica flakes  
or splittings coated with a binder formed by  
20 mixing boric acid, water and glycerin, and  
heating the superposed flakes or splittings  
to a temperature not exceeding 500° C.
11. A process of making composite mate-  
rial that comprises superposing mica flakes  
25 or splittings coated with a binder formed by  
mixing boric acid, water, glycerin and a  
pulverulent filler, and heating the super-
- posed flakes or splittings to a temperature  
not exceeding 500° C.
12. A binder for use in composite mate-  
rials comprising an oxygen compound of  
boron and a small amount of a pulverulent  
clay.
13. A binder for use in composite mate-  
rials comprising a compound of boron, a 35  
pulverulent clay filler and glycerin.
14. A binder for use in composite mate-  
rials comprising an oxygen compound of  
boron, a bentonite clay as a filler and glyc-  
erin. 40
15. The composite material resulting from  
subjecting to heat and pressure mica flakes  
or splits associated with a binder comprising  
an oxygen compound of boron and glycerin.
16. The composite material resulting from 45  
subjecting to heat and pressure mica flakes  
or splits associated with a binder comprising  
an oxygen compound of boron and a small  
amount of a pulverulent clay as a filler.
- In testimony whereof, I have hereunto 50  
subscribed my name this 27th day of Dec.,  
1916.

LEON McCULLOCH.